# EUROPEAN PATENT SPECIFICATION

(11) **EP 3 476 991 B1**
(45) Date of publication and mention of the grant of the patent: **14.04.2021**
(21) Application number: 17887808.8
(22) Date of filing: 15.12.2017
(51) Int. Cl.: D04H 3/105, D04H 3/011, D01D 5/098, D01D 5/22

(54) **METHOD FOR MANUFACTURING NON-WOVEN FABRIC FOR CARPET FOAM BACKING**
VERFAHREN ZUR HERSTELLUNG EINES VLIESSTOFFES FÜR TEPPICHSCHAUMSTOFFUNTERLAGEN
PROCÉDÉ DE FABRICATION DE TISSU NON TISSÉ POUR SUPPORT DE MOUSSE DE TAPIS

(30) Priority: 27.12.2016 KR 20160179842
(43) Date of publication of application: 01.05.2019
(73) Proprietor: Kolon Industries, Inc., Seoul 07793 (KR)
(72) Inventor: CHOI, Woo-seok, Gangseo-gu, Seoul 07793 (KR); LEE, Min-ho, Gangseo-gu, Seoul 07793 (KR); CHO, Hee-jung, Gangseo-gu, Seoul 07793 (KR); SEO, Hyok-jin, Gangseo-gu, Seoul 07793 (KR)
(74) Representative: Ter Meer Steinmeister & Partner
(86) International application number: PCT/KR2017/014819
(87) International publication number: WO 2018/124566

(56) References cited:
- EP-A1- 1 873 291
- JP-A- 2003 293 255
- JP-A- 2005 029 052
- JP-B2- 4 034 520
- KR-B1- 100 212 752
- KR-B1- 101 035 110
- US-A1- 2004 097 154
- DATABASE WPI Week 201527 Thomson Scientific, London, GB; AN 2015-24779N XP002797136, & KR 2015 0035138 A (KOLON IND INC) 6 April 2015 (2015-04-06)

## Description

### [Technical Field]

The present invention relates to a method of preparing a non-woven fabric for a base cloth of a carpet, which has an improved fixability of BCF (bulked continuous filament) yarn inserted on a base cloth in a tufting process for manufacturing a carpet.

### [Background Art]

Carpets are used not only for decoration in hotels, offices, homes, cars, but also for providing amenity and sound insulation.

The carpet fabric is manufactured through a process including a tufting step of introducing BCF yarn to a non-woven fabric and a back coating step of coating a solution such as PVC, PE, EVA or SBR, etc. the back side of the tufted non-woven fabric and curing. The carpet fabric is cut into squares (for example, 50 cm × 50 cm) to be used as tile carpets in hotels, offices, homes, etc., and molded in the form of a car floor to be used as a car floor mat.

The function of the base cloth of a carpet is to fix the BCF yarn.

In the tufting process, the base cloth is punctured by a needle to have open hole of at least 160,000 holes/m². The base cloth must maintain the arrangement of the BCF yarns in even though such physical damage and have no deformation of the shape in the post-process at the high temperature environment.

Recent trends in the tufting process are densification, diversification of pattern and the use of low denier BCF. For example, there is a tendency to increase the tufting density by using microfibers of BCF yarns, to make at least three BCF yarns at multilevel conditions, and to increase the movement of needles by using BCF yarns of various colors. Tufting becomes more difficult. Accordingly, the fixability of the BCF yarn in the non-woven fabric for base cloth has to be improved by increasing the coefficient of friction between the non-woven fabric and the BCF yarn so as to prevent the damage to the base cloth.

Meanwhile, conventional non-woven fabric for base cloth of carpet is produced by stretching and a thermal or chemical bonding of the filaments having potential stress. After that the residual stress of the filament is removed by heating in the post-processing for the manufacture of carpet, thereby exhibiting a high shrinkage ratio. Due to this, there is a problem that the shape of the final carpet product is deformed

KR 2015/0035138 and EP 1 873 291 both describe polyester needlefelts intended for use as base cloths for carpets.

### [Disclosure]

### [Technical Problem]

In order to solve the above problems, the present invention provides a method of preparing a non-woven fabric for a base cloth of a carpet, which has an increased fixability of BCF by improving a method of preparing a non-woven fabric for a base cloth a of carpet.

### [Technical Solution]

In order to solve the above-mentioned problems, the present invention provides a method of preparing a non-woven fabric for base cloth of a carpet comprising: preparing a stretched polyester filament fiber having a circular cross section; forming a web by integrating the filament fiber in a web form, crimp processing and calendering it; and needle punching the web, as defined in claim 1.

### [Advantageous Effects]

According to the present invention, the web with the stretched polyester filament is crimp processed and needle punched. By this the residual stress of the stretched polyester filament is eliminated and the formability is improved, and the fixability of the BCF yarn can be improved by interlacing polyester filament.

### [Best Mode]

The present invention relates to a method of preparing a non-woven fabric for a base cloth of a carpet comprising: preparing stretched filament to form a web, crimp processing and calendering and needle punching the web, as defined in claim 1.

The present invention further relates to a non-woven fabric for a base cloth of a carpet, as defined in claim 2.

The present invention may use filament fibers having a circular cross section and a low fineness such as 4 to 7 deniers, which is produced by melting a polyester having a melting point of at least 250 °C, discharging it through a spinneret to form a filament and stretching the filament to a spinning speed of 4,500 to 5,000 m/min using an air stretching device of high pressure.

In the present invention, when the fineness is less than 4 deniers, the damage of fibers occurs during tufting and the fixability of the BCF yarn may be deteriorated, and when the fineness is more than 7 deniers, the coefficient of friction may be lowered and it can be difficult to improve the pullout strength.

The flexibility of the filament is given by piling up the filament fibers on the conveyor in the form of a web and heating and crimp processing them.

The crimp processing is a processing method of heat treatment of synthetic fiber filament to form a thin curvature, and the yarn becomes curled and flexible accordingly.

In the present invention, the stretched filaments are piled up on a conveyor net and at the same time are treated at 100 to 150 °C for 30 to 60 seconds.

Since the residual stress of the stretched filament is removed by heating in the crimping process, the shrinkage rate of the filament is lowered and the shape stability can be improved. Further, since the filament constituting the non-woven fabric is provided with a crimp and has a high coefficient of friction, and finally the fixability of the BCF yarn can be improved.

The number of crimps of the polyester filament fiber in the crimping process is 20 to 40 per 2.54 cm (20 to 40 per inch). At this time, if the number of crimps is less than 20 per 2.54 cm (20 per inch), the contact points between the filaments are decreased and the strength and elongation of the non-woven fabric after calendering or needle punching are lowered, and the force to fix the BCF yarn after tufting is weakened. When the number of crimps exceeds 40 per 2.54 cm (40 per inch), the contact points become too large and the filaments may be damaged due to excessive adhesion between the filaments during needle punching and the coefficient of friction of the non-woven fabric is too high, thus BCF yarn with a low fineness may be damaged when tufting.

Thereafter, a non-woven fabric in which interlacing is formed between the filaments can be produced by passing crimp processed web through a calendering roll to adjust its thickness and needle punching it.

According to the calendering of the present invention, it has a thickness of 0.35-0.50 mm by applying a predetermined temperature (130-150 °C) and pressure to reduce the thickness of the non-woven fabric. Accordingly, the density increases and the amount of filament for interlacing increases.

Needle punching is performed in two steps. The first step (pre-punching) is performed in the condition of 300 to 400 stroke rpm (the speed at which the non-woven fabric is bonded by the needle during passing through the conveyor net) to form a web shape by interlacing a portion of the filament. In the second step (main punching), the filaments are interlaced entirely with a condition of 600 to 800 stroke rpm to produce a non-woven fabric for base cloth of carpet.

In the non-woven fabric for base cloth of carpet produced as described above, the potential stress of the amorphous region oriented in the stretched filament is eliminated by the crimp processing. In the subsequent process, the shrinkage rate is reduced due to heat and the curvature is formed to increase the interlacing point of the filament. Thus, increased tensile strength and tear tension of the non-woven fabric may exhibit in the needle punching process.

Hereinafter, the present invention will be described in more detail with reference to the following Examples and Comparative Examples.

It should be noted, however, these embodiments of the present invention have been described for illustrative purposes, and therefore, the present invention is not limited thereto, and it will be apparent to those skilled in the art that modifications and variations could be made without departing from the scope of the present invention as defined by the appended claims.

### <Example 1>

Polyethylene terephthalate (PET) for fibers having a melting point of 260 °C was melted in an extruder at 288 °C and discharged through capillaries of the spinneret. The discharged PET was solidified by using a cooling wind, and then stretched using a stretching device and spun at a spinning speed of 5,000 m/min. Thus, filament fiber having a circular cross section with a fineness of 6 denier was produced.

The crimp processing was performed such that the filament fiber was piled up on a conveyor net in form of a web and simultaneously the stacked filament was heated at 130 °C for 60 seconds to form a crimp number as shown in the following Table 1.

Thereafter, the calendering was carried out by passing through a heated calendering roll to have smoothness and appropriate thickness to the non-woven fabric.

Then, the needle punching of the first and second steps were performed in the conditions shown in Table 1 below to produce a non-woven fabric for base cloth of carpet having an interlaced filament and a weight per unit area of 120 g/m².

### <Examples 2 to 4>

A non-woven fabric for base cloth of carpet was prepared by the same method as the Example 1, except that crimp processing and needle punching were carried out in the conditions shown in Table 1 in the Example 1.

### <Comparative Examples 1 to 4>

A non-woven fabric for base cloth of carpet was prepared by the same method as the Example 1, except that crimp processing and needle punching were carried out in the conditions shown in Table 1 in the Example 1.

**[Table 1]**

| Example | Crimp number | First step needle punching condition (stroke rpm) | Second step needle punching condition (stroke rpm) |
|---|---|---|---|
| Example 1 | 20 | 350 | 700 |
| Example 2 | 30 | 350 | 700 |
| Example 3 | 40 | 350 | 700 |
| Example 4 | 30 | 350 | 800 |
| Comparative Example 1 | 15 | 350 | 700 |
| Comparative Example 2 | 30 | 350 | 500 |
| Comparative Example 3 | 50 | 350 | 700 |
| Comparative Example 4 | 30 | 350 | 900 |

The Examples and Comparative Examples were evaluated by the following evaluation methods and the results thereof are shown in the following Table 2.

### <Evaluation method>

### 1. Tensile strength (kgf/5 cm) and elongation (%)

KS K 0521 method was used. A specimen having a size of length × width = 5 cm × 5 cm was measured by a measuring instrument of Instron with fixing by a jig having upper/lower 5 cm x 5 cm at a tensile speed of 200 mm/min.

### 2. Formability

After applying PVC solution on the back of the non-woven fabric and drying it, a lattice pattern with gap of 2 cm is drawn on the specimen having a size of length × width = 50 cm × 50 cm. Thereafter, the non-woven fabric is preheated at 180 °C for 3 minutes in a preheating plate and the molding is performed using a square mold having a size of 20 cm x 20 cm with the engraved lower plate and the embossed upper plate. After molding, the number of lattice patterns at the torn portion in the non-woven fabric was counted to obtain the width of the torn portion.

### Ex) Number of cells in torn area = 2 cells = 2 × 2 = 4

### 3. Pullout strength (gf)

Loft type tufting is performed at a speed of 800 rpm under the condition of 10 needles per inch in the width direction and 13 needles per inch in the length direction when tufting. After tufting, one adjacent loop to the loop to be measured is cut off and a loop with 10 loops apart on the opposite side is cut off. An average of 10 intensity peaks appearing when the loops to be measured are pulled in a direction perpendicular to that of the non-woven fabric using an Instron is calculated. The number of specimens is three.

**[Table 2]**

| | Tensile strength (MD/CD, kgf/5cm) | Tensile elongation (MD/CD, %) | formability (cm×cm) | Pullout strength (gf) | Overall evaluation |
|---|---|---|---|---|---|
| Example 1 | 14.1/15.7 | 34.2/35.9 | 0 | 2.1 | ○ |
| Example 2 | 15.9/16.3 | 31.4/34.3 | 0 | 2.6 | ⊚ |
| Example 3 | 18.8/20.7 | 28.3/29.2 | 0 | 2.8 | ⊚ |
| Example 4 | 17.3/18.8 | 29.4/30.1 | 0 | 2.7 | ⊚ |
| Comparative Example 1 | 10.1/12.5 | 40.6/37.4 | 7 | Tufting impossible | × |
| Comparative Example 2 | 14.3/15.1 | 30.3/34.7 | 3 | 2.3 | Δ |
| Comparative Example 3 | 23.8/24.7 | 38.9/37.6 | 4 | 2.4 | Δ |
| Comparative Example 4 | 10.8/11.7 | 39.8/38.1 | 15 | Tufting impossible | × |

From the results of the Table 2, when the number of crimps of the filaments constituting the non-woven fabric was small (Comparative Example 1), tufting was impossible. It is considered because the number of contact points was small and the friction coefficient was improved with minimal compared with Example 1. When the number of crimps of the filaments is large (Comparative Example 2), the mechanical strength is improved, but the non-woven fabric becomes stiff and the formability is declined.

When the needle punching was excessive (Comparative Example 4), tufting was impossible, which is confirmed by the damage of the filament. When the needle punching is performed in small degree (Comparative Example 2), the mechanical strength is not improved and the formability is lowered.

### [Industrial Applicability]

From the above, it can be seen that the non-woven fabric according to the present invention is improved in formability and pullout strength in the process of preparing a carpet, thereby contributing the improvement of productivity and quality of the carpet.

## Claims

1. A method of preparing a non-woven fabric for a base cloth of a carpel comprising:
preparing a stretched polyester filament fiber having a circular cross section forming a web by integrating the filament fiber in a web form, crimp processing and calendering it; and
needle punching the web,
wherein the crimping processing is performed such that the stretched filament fiber is piled up on a conveyor net for forming the web and at same time, the stretched filament is treated at 100 to 150 °C for 30 to 60 seconds to form number of crimps of 20 to 40 per 2.54 cm (20 to 40 per inch), and
wherein the needle punching is performed in a first step and a second step and in a condition of 300 to 400 stroke rpm in the first step and 600 to 800 stroke rpm in the second step.

2. A non-woven fabric for a base cloth of a carpet prepared by the method of claim 1, which comprises a polyester filament fiber having a monofilament fineness of 0.44 to 0.78 mg/m (4 to 7 denier), and has a pullout strength of 0.20 to 0.03 N (2.0 to 3.0 gf) (strength to pull loop after loop type tufting) in the non-woven fabric,
wherein the pullout strength is measured by loof type tufting which is performed at a speed of 800 rpm under the condition of 10 needles per inch in the width direction and 13 needles per inch in the length direction when tufting, and after tufting, one adjacent loop to the loop to be measured is cut off and a loop with 10 loops apart on the opposite side is cut off, and an average of 10 intensity peaks appearing when the loops to be measured are pulled in a direction perpendicular to that of the non-woven fabric using an Instron is calculated.

## Patentansprüche

1. Verfahren zum Herstellen eines Vliesstoffs für ein Grundgewebe eines Teppichs, umfassend:
Herstellen einer gestreckten Polyesterfilamentfaser, die einen kreisförmigen Querschnitt aufweist;
Ausbilden einer Bahn durch Einbringen der Filamentfaser in eine Bahnform, einer Kräuselvearbeitung und einem Kalandrieren derselben; und
Nadel stanzen der Bahn,
wobei eine Kräuselvearbeitung derart durchgeführt wird, dass die gezogene Filamentfaser auf einem Transportnetz zum Ausbilden der Bahn aufgestapelt wird und gleichzeitig das gezogene Filament bei 100 bis 150 °C 30 bis 60 Sekunden lang behandelt wird, um eine Anzahl von Kräuselungen von 20 bis 40 pro 2,54 cm (20 bis 40 pro Zoll) auszubilden, und
wobei das Nadelstanzen in einem ersten Schritt und einem zweiten Schritt und in einem Zustand von 300 bis 400 Hubumdrehungen pro Minute in dem ersten Schritt und 600 bis 800 Hubumdrehungen pro Minute in dem zweiten Schritt durchgeführt wird.

2. Vliesstoff für ein Grundgewebe eines Teppichs, der durch das Verfahren nach Anspruch 1 hergestellt wird, der eine Polyesterfilamentfaser umfasst, die eine Monofilamentfeinheit von 0,44 bis 0,78 mg/m (4 bis 7 Denier) aufweist und eine Ausreißkraft von 0,20 bis 0,03 N (2,0 bis 3,0 gf) (Kraft, um die Schlaufe nach dem Schlaufentuften zu ziehen) in dem Vliesstoff aufweist,
wobei die Ausreißkraft durch Schlaufentuften gemessen wird, das bei einer Geschwindigkeit von 800 Umdrehungen pro Minute unter der Bedingung von 10 Nadeln pro Zoll in der Breitenrichtung und 13 Nadeln pro Zoll in der Längenrichtung beim Tuften durchgeführt wird, und nach dem Tuften eine angrenzende Schlaufe zu der Schlaufe, die gemessen werden soll, abgeschnitten wird und eine Schlaufe mit 10 Schlaufen Abstand auf der gegenüberliegenden Seite abgeschnitten wird, und ein Durchschnitt von 10 Intensitätsspitzen, die auftreten, wenn die Schlaufen, die gemessen werden sollen, in einer Richtung senkrecht zu der des Vliesstoffs gezogen werden, unter Verwendung eines Instrons berechnet wird.

## Revendications

1. Procédé de préparation d'une étoffe non tissée pour un tissu de base d'une moquette comprenant :
la préparation d'une fibre de filaments de polyester étirés ayant une section transversale circulaire;
formant une voile en intégrant la fibre de filaments sous une forme de voile, en la traitant par frisure et en la calandrant ; et
l'aiguilletage de la voile,
dans lequel le traitement par crêpage est effectué de telle sorte que la fibre de filaments étirés est empilée sur un filet de convoyeur pour former la voile et en même temps, le filament étiré est traité de 100 à 150 °C pendant 30 à 60 secondes pour former un nombre de frisures de 20 à 40 par 2,54 cm (20 à 40 par pouce), et
dans lequel l'aiguilletage est effectué au cours d'une première étape et d'une seconde étape et dans une condition de 300 à 400 tr/min de course au cours de la première étape et de 600 à 800 tr/min de course au cours de la seconde étape.

2. Étoffe non tissée pour un tissu de base d'une moquette préparée par le procédé de la revendication 1, qui comprend une fibre de filaments de polyester ayant une finesse de monofilament de 0,44 à 0,78 mg/m (4 à 7 deniers), et a une résistance à l'arrachement de 0,20 à 0,03 N (2,0 à 3,0 gf) (résistance à la traction de la boucle après le tuftage de type boucle) dans l'étoffe non tissée,
dans lequel la résistance à l'arrachement est mesurée par un tuftage de type boucle qui est effectué à une vitesse de 800 tr/min dans la condition de 10 aiguilles par pouce dans le sens de la largeur et de 13 aiguilles par pouce dans le sens de la longueur lors du tuftage, et après le tuftage, une boucle adjacente à la boucle à mesurer est coupée et une boucle avec 10 boucles écartées du côté opposé est coupée, et une moyenne de 10 pics d'intensité apparaissant lorsque les boucles à mesurer sont tirées dans une direction perpendiculaire à celle de l'étoffe non-tissée à l'aide d'un système Instron est calculée.
